

Nov. 10, 1931.

A. THOMA

**1,831,269**

## ANTISQUEAK MATERIAL FOR SHOES

Filed Aug. 8, 1927



35 F<sup>r</sup> C<sup>o</sup>. 12. 33 F Inventor  
Andrew Thomas  
25<sup>a</sup> F<sup>r</sup> C<sup>o</sup>. 13. 24<sup>a</sup> F<sup>r</sup> C<sup>o</sup>. 14. 24<sup>b</sup> By Robert Cushman Woodbury  
3<sup>b</sup> By Attorneys

## UNITED STATES PATENT OFFICE

ANDREW THOMA, OF CAMBRIDGE, MASSACHUSETTS, ASSIGNOR TO NORTH AMERICAN CHEMICAL COMPANY, OF BOSTON, MASSACHUSETTS, A CORPORATION OF MASSACHUSETTS

## ANTISQUEAK MATERIAL FOR SHOES

Application filed August 8, 1927. Serial No. 211,300.

This invention pertains to the manufacture of footwear and more particularly to means for eliminating squeak-producing friction between the parts of a shoe and to a method or process of producing such anti-squeak means.

According to most processes of manufacture, the various elements constituting the bottom of a shoe are united only along the marginal portion of the bottom, thus providing the desired flexibility for the comfort of the wearer, but the slight relative movement and rubbing of the shoe parts mainly within the boundary of said margin or within the marginal line of stitches or other fastenings which is thus permitted, frequently results in producing a disagreeable squeak. This is especially noticeable in shoes of the McKay type, (where a large portion of the bottom of the inner sole is covered by the folded-over edge of the upper) and in shoes of any type in which a dry (non-adhesive) filler is interposed between the outer sole and contiguous parts. When the outer sole is fastened in place it bears against these folded-over edge portions of the upper, and the filler material, and as the wearer flexes the shoe in walking the parts rub and a squeaking noise results.

In accordance with the present invention I interpose an anti-friction or anti-squeak element between those parts of the shoe which have hitherto tended to rub and squeak, preferably providing this anti-squeak element in a form such that it is easy and cheap to make, readily packed for storage or shipment (if necessary), which can be applied to the shoe without the aid of special machinery or equipment, and which does not affect the other and usual steps in the shoe-making process or substantially change the appearance or weight of the completed shoe.

A preferred form of anti-squeak element consists of a sheet of paper, paper-like substance, textile fabric or any other suitable sheet material, having sufficient toughness and flexibility and of proper thickness for the purpose, such sheet being coated and preferably impregnated with a sticky and desirably waterproof or water-repellent substance and in the latter case preferably loaded or filled with a powdered mineral anti-squeak element.

While I obtain good results by the interpolation of such a sticky sheet or layer between shoe parts, I prefer to dust or otherwise coat this sticky sheet with an anti-friction powder or other slippery substance which sticks to and is held in place by the sticky coating of the base fabric. This powder imparts to the base fabric a smooth, slick surface which does not adhere to adjacent parts of the shoe and which is so slippery that squeak-producing friction is impossible. The waterproofed sheet with its sticky surface (of wax tailings for instance) is thus rendered non-sticky by the talc or other mineral powder, producing a film or layer of paste or putty-like consistency as a mechanical lubricant. Heretofore talc has occasionally been used dry between the two soles and has quickly been lost so far as the anti-friction or anti-squeak effect was concerned. I provide the film stated, or layer or coating which is therefore immovable and hence not to be lost in use. The more this layer of powder is rubbed the better it will stay in place and the more securely it will be bound to the paper, because a rubbing pressure on the layer of powder tends to force it somewhat into the surface of the permanently sticky binder with which the paper or carrying layer is impregnated or coated, thus strengthening the bond between the layer of powder and the layer of paper. The sticky absorbent is itself an excellent anti-squeak element.

In order that the anti-squeak material may not lose its effectiveness I regard it as important that the sticky coating or impregnant employed be of such a nature that it will retain its stickiness and tenacity indefinitely. In certain prior patents relating to shoe filler compounds, for example my Patent Nos. 808, 85 224, December 6, 1905; 832,002, September 25, 1906; and 855,868, June 4, 1907, I have described various forms of permanently sticky binder materials, all of which possess characteristics making them more or less acceptable for the present purpose. However, by reason of its relative cheapness, availability and highly adhesive properties, I prefer to employ a coating or impregnating material comprising the sticky residuum of petroleum 100

known as wax-tailings, or combinations thereof with oils, resins, pitches or gums as more fully described for example in my Patent No. 855,868.

5 In coating or impregnating the sheet material I find it convenient to provide such material in the form of a web of considerable length and of desired width, and I draw this web of fabric lengthwise through a bath of the coating or impregnating material,—scraping off or otherwise removing surplus material as the web leaves the bath. In employing wax tailings or similar materials I find it desirable to heat the bath to make its 15 constituents more fluid and penetrative of the fabric, and I sometimes subject the web to pressure within the bath or after leaving the bath in order to force the coating or impregnating material into the pores of the web.

20 The sheet material thus treated has a thin surface coating or film of a permanently sticky character, waterproof and strongly adhesive to leather, and this sheet material may be interposed in this condition between 25 those elements of the shoe which commonly rub and squeak. When thus used the thin, permanently sticky, waxy and elastic film or coating of the sheet tends to adhere to the shoe parts with which it contacts and forms a 30 yielding cushion for the latter. As the shoe parts move relatively, this thin, elastic, waxy film yields, although apparently still maintaining its grip upon the shoe parts, and behaves like a lubricant fluid body, becoming 35 warm (and incidentally more sticky) through internal friction but exhibiting no tendency to mechanical vibration of a kind which will produce a squeak.

40 While the coated or impregnated fabric may thus be used without further treatment, its sticky surface makes it somewhat hard to handle and particularly to ship or store, and I thus prefer to provide a protective coating for the sticky sheet material. While a coating intended to be stripped off or otherwise 45 removed, prior to application of the anti-squeak element to the shoe may be provided, I prefer to employ a coating as above suggested which may form a permanent part of 50 the anti-squeak element and which is preferably of such a nature as to enhance the anti-squeak properties of the sticky coating material. To this end I dust or otherwise spread an anti-friction powder upon one or 55 both of the sticky surfaces of the sheet material, such powder preferably being of an unctuous nature, for example graphite, a powdered mineral, such as talc or soapstone, or a slippery non-absorbent flaky material, 60 such for example as powdered mica.

65 When thus treated, the powder dulls the normal stickiness of the outer surface of the coated material but the sticky coating holds the powder layer firmly in place and while 75 the shoe-elements normally slip in contact

with the slick, smooth surface of the powder layer, the normal elasticity and yielding character of the sticky coating is substantially unimpaired and acts as an elastic lubricating cushion with respect to the dust layer in the 70 same way as when it is applied directly to the shoe parts.

In the accompanying drawings I illustrate by way of example certain steps comprised in a desirable process of making my anti-squeak 75 material, together with various modes of coating and applying this material to a shoe, but without intending thus to limit my invention.

In the drawings:

Fig. 1 is a diagrammatic elevation, partly in section, showing apparatus suitable for use in preparing my anti-squeak material in sheet form;

Fig. 2 is a fragmentary vertical section, to 85 very large scale, illustrative of the character of the sheet material resulting from the complete process indicated in Fig. 1;

Fig. 3 is a fragmentary plan view illustrating one mode of cutting anti-squeak elements 90 from the sheet material;

Fig. 4 is a plan view of one of the elements cut as indicated in Fig. 3;

Figs. 5 and 6 are plan views illustrating modified shapes of anti-squeak elements; 95

Figs. 7, 8 and 9 are plan views illustrating another mode of preparing anti-squeak elements from sheet material;

Fig. 10 is a fragmentary plan view, partly in perspective, illustrating the application of 100 the anti-squeak element of Fig. 4 to a McKay shoe;

Fig. 11 is a similar view illustrating the application of the anti-squeak element of Fig. 5 to a McKay shoe;

Fig. 12 is a transverse section, substantially on the line 12—12 of Fig. 10, but to larger scale, showing the outer sole of the shoe in place; and

Figs. 13 and 14 are fragmentary vertical 110 sections to large scale showing modified forms of anti-squeak sheet material.

Referring to Fig. 1, the numeral 1 designates a spindle or roller upon which is mounted a roll 2 of sheet material, such for example as a web of paper, textile fabric or the like. This sheet material 3 passes from the roll to a receptacle 4, preferably provided with guide rolls 5 and 6 adjacent to its opposite edges, and with rollers 7 and 8 in its 115 lower part for guiding the sheet 3 downwardly into the receptacle. If desired one or both pairs of rolls 5 and 6, or 7 and 8, may be positively driven and preferably the rolls 7 and 8 are arranged to exert a substantial 120 pressure upon the sheet 3 as it passes between them.

The receptacle or tank 4 is preferably provided with heating means, as for example the steam coils 9, and is adapted to contain a 130

body 10 of coating or impregnating material of the kind above referred to, and which is permanently sticky and very elastic, for example, wax tailings.

- 5 On its way from the rolls 7 and 8 to the delivery rolls 6, the web passes between scraper devices 11 which remove the surplus coating and impregnating fluid, and the web or sheet 3 may then pass to a guide roll 12. 10 On its way to this guide roll the web passes beneath a receptacle 13 containing a slippery inert powder, such for example as graphite, talc, soapstone, powdered mica or the like, and this material may be spread upon one 15 sticky surface of the web by brush 14 or any other suitable means. From the guide roll 12 the web passes under a guide roll 15 and beneath a receptacle 16 containing a slippery powder of the same kind as used in said receptacle 13, which is dusted upon the other sticky surface of the web by means of a brush 17. Thus both surfaces of the web are 20 coated with the powder.

From this point the web may pass between 25 rolls 18 which, if desired, exert some pressure in order to embed the powder in the sticky coating, and then the web may be passed about guide rolls 19 to form festoons 20, if desired, to furnish a sufficient time interval for the impregnant to cool and harden. The completed sheet material S, comprising 30 the original web with its surface coatings, may now be rolled upon a spindle 21 to form a roll 22, or may be cut into sheets of suitable size or handling, packing, etc.

In Fig. 2 the completed sheet S (in enlarged section) is shown as comprising the original web or sheet 3 having the sticky coatings 24 on its opposite sides to which the layers 25 of powder adhere. During the 35 passage of the web through the bath of fluid coating material 10, the fluid tends to enter the pores of the web, particularly if the web be subjected to pressure, thus impregnating the web and rendering it waterproof.

The sheet material thus prepared may now be cut up in any desired manner, and when to be used in a shoe the sheet S, as indicated in Fig. 3, may be cut into sections 26 by 40 means of suitable dies, such sections having a contour substantially like that of the forepart of a shoe bottom and being adapted to cover the central portion of the inner sole of a shoe as well as preferably the marginal portions of the bottom.

In Fig. 5 I have indicated a modification in which the anti-squeak element 27 has a contour similar to that of the shoe bottom but is cut out at its central portion so that 45 it covers only the marginal portions of the shoe bottom. In Fig. 6 I have shown a curved piece 28 of the sheet material which is adapted to cover the marginal portion of the shoe bottom at one side and which must 50 be associated with similar sections in order

to extend around the entire margin of a shoe. This shape of anti-friction element may be desirable for the sake of economy in cutting.

In Fig. 7 I have shown a straight strip 29 of the sheet material and in Fig. 8 I have 55 shown a similar strip 30 notched at 31 along one edge to facilitate its bending to enable it to follow the contour of the shoe bottom. This strip 30, bent so as to conform to the edge of a shoe bottom, is shown in Fig. 9.

In Figs. 10 and 12 I have indicated diagrammatically and in section respectively a shoe of the McKay type comprising the upper U and the inner sole 33—the edge portions 34 of the upper being turned inwardly and folded down upon the under surface of the inner sole to which these edge portions of the upper are secured by means of fasteners F. The central cavity of the shoe bottom, defined by the edges of the upper, is provided with filler 35 which may be of any usual material and upon this filler rests the anti-squeak element 26 of the kind shown in Fig. 4. Preferably I apply adhesive to the central portion of the anti-squeak element 26 before applying it to the shoe bottom, the adhesive area being indicated at 27. After applying the anti-squeak element in this manner, the outer sole 36 is 60 placed in position and secured by means of 90 stitches 37 or other usual form of fastener.

The thin sheet-like anti-squeak element 26, consisting of the inner web of paper-like material and the outer coatings of slippery powder permanently held in position by the sticky layers 24, forms a very effective preventive of friction, such as would cause squeaking, since the outer sole bears against one slippery and unctuous layer 25 while the inturned edge portions 34 of the upper bear 65 against the other slippery layer 25. Thus even though the shoe parts have some relative movement, they are free to slide without setting up mechanical vibrations such as would produce a noise, and even though 100 it were possible for the shoe parts to adhere to the slippery layers, the latter are supported upon the cushioning and lubricating layers of sticky material which is elastic and stretches readily and which, being of semi-fluid character, will not squeak when subjected to rubbing pressure.

By reason of the waterproof qualities of this anti-squeak material its interposition between the bottom elements of the shoe tends 105 to waterproof the latter and to prevent moisture from passing through the outer sole into the inner sole.

In Fig. 11 I have shown a shoe similar to that indicated in Figs. 10 and 12, but having the anti-squeak element 27 applied thereto, instead of the element 26. This anti-squeak element 27 extends around the marginal portion of the shoe bottom and is interposed between the outer sole and the inturned por- 120 125 130

tion of the upper so that it effectually prevents frictional rubbing of these parts.

While I have described my anti-squeak material as consisting of a web coated on both sides with a sticky substance and a slippery powder, I contemplate that for some purposes it may be desirable to coat but one side of the web and in these or other circumstances it may be preferable merely to coat the web rather than to attempt to impregnate it.

I further contemplate that within the scope of my invention I may omit the base fabric or web 3 and provide an anti-squeak element 15 consisting, as indicated in Fig. 13, merely of one or more layers 25<sup>a</sup> of non-adhesive powder or dust embedded in a layer 24<sup>a</sup> of sticky material. On the other hand, as already suggested, and as shown in Fig. 14, 20 I may omit the slippery powder altogether and form my anti-squeak material of a sheet or web 3<sup>b</sup> coated on one or both sides (and impregnated, if desired) with a sticky material, as shown at 24<sup>b</sup>.

25 While I have described one desirable mode of making my anti-squeak material and have indicated several ways of coating this material and applying it to shoes, I wish it to be understood that this is merely by way of 30 illustration and is not intended to limit the scope of the invention, but that I contemplate that the material may be made in accordance with other sequences of steps, that it may be cut and applied to shoes in other 35 ways than those herein specifically suggested.

I claim:

40 1. Anti-squeak material for use in shoes, said material being permanently flexible and comprising a thin layer of slippery powder and a thin layer of a permanently sticky elastic substance.

2. Anti-squeak material for use in shoes, said material comprising a thin sheet of paper, a layer of powdered talc and sticky wax tailings binding the talc to the paper.

3. A permanently flexible anti-squeak element for use in shoes having an outer contour substantially conforming to the outer contour of a shoe bottom and comprising a thin sheet of paper having a permanently sticky coating including wax tailings.

4. Anti-squeak material for use in shoe bottoms, comprising a thin, flexible, non-plastic base sheet, an outer layer of slippery powder and permanently flexible and sticky adhesive means for binding the powder layer to the base sheet.

5. Anti-squeak element for use in shoe bottoms, said element comprising a thin permanently flexible non-plastic base sheet and a layer or coating of permanently sticky substance on one outer face at least of the base sheet, said element being of such thickness as to adapt it for insertion between the outer sole

of a shoe and all parts of the shoe bottom which normally would contact with the outer sole but without substantially increasing the vertical dimensions of the shoe.

6. An anti-squeak element for use in shoes, 70 said element consisting of a thin sheet of substantially uniform thickness throughout comprising a permanently sticky substance, said element being permanently flexible and having an outer contour such as to conform closely to the outer edge of the bottom of a shoe with which it may be associated, and a layer of slippery powder substantially covering each outer face of said element.

7. An anti-squeak element for use in shoes, 80 said element consisting of a thin sheet of a thickness adapting it for insertion between the outer sole of a shoe and all parts of the shoe bottom which would normally contact with the outer sole, said sheet being permanently flexible and comprising a permanently sticky substance having a normal tendency to adhere to the outer sole and to the opposed parts of the shoe bottom.

8. An anti-squeak element for use in shoes, 90 having such thickness as to be included between the outer sole of a shoe and other parts of the shoe bottom without substantially increasing the vertical dimensions of the shoe, said element comprising a layer of permanently sticky substance having a normal tendency to adhere to the outer sole and to the opposed parts of the shoe bottom.

9. An anti-squeak element for use in shoes, 100 having such thickness as to be included between the outer sole of a shoe and other parts of the shoe bottom without substantially increasing the vertical dimensions of the shoe, said element comprising a layer of permanently sticky substance and a layer of slippery powder. 105

Signed by me at Boston, Massachusetts, this 5th day of Aug. 1927.

ANDREW THOMA.

110

115

120

125